

Aug. 21, 1934.

B. LONG

1,971,268

PROCESS OF AND APPARATUS FOR TEMPERING GLASS SHEETS

Filed June 17, 1932



FIG. 1.



FIG. 2.



FIG. 3.



FIG. 4.



FIG. 5.

Inventor

BERNARD LONG

By

Dorsey Cole

Attorney

## UNITED STATES PATENT OFFICE

1,971,268

## PROCESS OF AND APPARATUS FOR TEMPERING GLASS SHEETS

Bernard Long, Paris, France, assignor, by mesne assignments, to The American Securit Company, a corporation of Delaware

Application June 17, 1932, Serial No. 617,891  
In France July 24, 1931

6 Claims. (Cl. 49—45)

In my prior U. S. applications, Serial No. 434,263, filed March 8, 1930; and Serial No. 567,286, filed October 6, 1931, I have described a process of tempering glass sheets by projecting 5 jets of air under pressure thereon while the sheet is heated. The present application has for its object to accomplish the tempering by jets of air or another gaseous fluid, produced not by a pressure applied to the air before striking the plate, 10 but by a reduction in air pressure adjacent to the plate, so that the air adjacent to the latter is rapidly removed therefrom. This I accomplish by placing the sheet to be tempered in an enclosure and connecting the enclosure with suitable 15 means for aspirating or withdrawing the air therefrom, the enclosure having ports in its side walls through which external air enters to strike the plate and to produce a surface chilling there- 20 of.

Referring to the accompanying drawing in which corresponding parts are designated by corresponding marks of reference,—

Fig. 1 is a vertical transverse section showing an apparatus embodying my invention and suitable 25 for carrying out the process herein described and claimed.

Figs. 2 and 3 are views similar to Fig. 1, illustrating modifications thereof.

Figs. 4 and 5 are side elevations of the device 30 shown in Fig. 2.

In all forms of the invention here disclosed the glass sheet *b* is hung by suitable tongs *c* within a suitable enclosure *a*, which may be of sheet iron, and which has generally flat sides which conform 35 with more or less exactness to the shape of the sheet and are parallel to the faces thereof. The tongs are supported by a hanger *d* carrying a closure plate *f* adapted to seal the otherwise upper open end of the enclosure *a*. To the base of the 40 enclosure *a* a suitable aspirating pipe *k* is connected and the side walls *g* of the enclosure are provided with ports *h*.

With such a construction, when a sheet *b* which has received a proper preliminary heat treatment 45 such as is described in my prior applications is placed within the enclosure and the tongs *c* lowered to close the upper end of the enclosure, air is drawn from the interior of the enclosure through the pipe *k* to reduce the pressure there- 50 in. This air is replaced by air external to the enclosure entering through the ports *h* and striking the sides of the sheet to temper the same. It has been found that advantages result from the reduction of pressure adjacent the sheet over 55 what happens when the air is blown by superat-

mospheric pressure against the sheet. It is obvious that the arrangement of the ports *h* in the walls *g* of the enclosure may be selected with a view of obtaining the desired distribution of cooling centers.

In Fig. 2 an arrangement is shown better suited than that of Fig. 1 for sheets of larger size. In this arrangement air eduction pipes *k'* and *k''* are connected with the top of the enclosure so that air is withdrawn from both the top and bottom thereof. Moreover, a slide damper *r* is arranged adjacent to each side wall of the enclosure and is provided with ports *s*, (see Figs. 4 and 5) the arrangement of the ports *s* in the damper being such that in one position of the damper one group of ports *g* in the side wall of the enclosure is uncovered, while in another position of the damper the other group of ports *g* is uncovered. Thus, by reciprocating the damper two groups of chilling centers are provided, as is described in my previous application, Serial No. 567,286.

In Fig. 3 an arrangement is shown for pre-chilling the air or another gas admitted through the ports *h*. This is accomplished by constructing chambers *l* upon the outside of the enclosure *a* along the side walls thereof and placing in such chambers pipe coils *p* through which a proper refrigerant may be circulated. Air for chilling is thus admitted into the interior of the enclosure from the chambers *l* and those chambers are replenished in their air supply through ports *n* located in their walls *m*.

Having thus described my invention what I claim and desire to secure by Letters Patent is:—

1. The hereinbefore described process of tempering glass plates which consists in creating air blasts against the plate by a zone of sub-atmospheric pressure surrounding the plate.

2. The hereinbefore described method of tempering glass which comprises creating a zone of sub-atmospheric pressure surrounding the glass and admitting air or another gas under substantially atmospheric pressure to such space through ports opposite to the surface of the plates.

3. In a device for tempering glass sheets, the combination with an enclosure having substantially parallel perforated sides, of means for suspending a glass sheet therein, and means for creating a sub-atmospheric pressure therein.

4. In a device for tempering glass sheets, the combination with an enclosure having parallel side walls with groups of perforations therein, means for suspending a plate within the enclosure, means for withdrawing air from the enclosure,

sure, and means for alternately opening and closing the several groups of apertures.

5. In a device for tempering glass sheets, the combination with an enclosure having a chilling chamber on each side thereof, separated from the interior of the enclosure by a perforated wall, means for suspending a glass sheet in the enclosure, and means for withdrawing air from the interior of the enclosure.

10

6. The hereinbefore described process of tempering a glass plate suspended vertically, which comprises maintaining a zone of sub-atmospheric pressure surrounding the plate while admitting jets of air or other gas under atmospheric pressure on selected points distributed over both faces of the plate.

80

BERNARD LONG.

85

15

90

20

95

25

100

30

105

35

110

40

115

45

120

50

125

55

130

60

135

65

140

70

145

75

150